

1

3,761,278

### SILVER HALIDE ELEMENT CONTAINING A BENZIMIDAZOLINE - 2 - THIONE-N,N'-DICARBONIC ACID ESTER STABILIZING AGENT

Walter Gauss, Cologne, Anita von Konig and Franz Moll, Leverkusen, Wolfgang Muller-Bardorff, Cologne, and Wilhelm Saleck, Schildgenberg-Gladbach, Germany, assignors to Agfa-Gevaert Aktiengesellschaft, Leverkusen, Germany

No Drawing. Filed Aug. 25, 1971, Ser. No. 174,930  
 Claims priority, application Germany, Aug. 27, 1970,  
 P 20 42 533.8; June 18, 1971, P 21 30 031.2  
 Int. Cl. G03c 1/34

U.S. Cl. 96—109

3 Claims

#### ABSTRACT OF THE DISCLOSURE

A photographic silver halide emulsion containing a fog-stabilizing amount of a benzimidazole-2-thione-N,N'-dicarbonic acid ester.

The invention relates to a photographic material comprising at least one silver halide emulsion layer the photographic properties of which have been improved by the addition of benzimidazole - 2-thione-N,N'-dicarbonic acid esters.

As is well known, light-sensitive silver halide emulsions, especially those which have been chemically sensitized, tend to the formation of fog, i.e. nuclei which are capable of undergoing development without exposure. Fogging occurs especially at high temperatures and atmospheric humidity, if development is carried out for too long or at too high temperatures, if certain additives are used or if the emulsions are too strongly ripened, etc. The tendency of photographic silver halide emulsions to fogging can be suppressed to a certain extent by the addition of so-called stabilizers or antifogging agents. Compounds which have this effect are e.g. heterocyclic mercapto compounds or inorganic or organic mercury compounds. The stabilizers have, however, the disadvantage that when used in effective concentrations they generally reduce the sensitivity of the stabilizing emulsions.

Another kind of fog is frequently formed in photographic materials comprising a paper support in particular a baryta-coated paper support. Upon processing of exposed photographic paper materials especially mechanical processes, thiosulfate frequently is carried from the fixing bath into the developing bath. In other cases, such as rapid-, stabilizing- or fixing developing baths, a silver halide solvent, e.g. thiosulfate is added to the developing bath. When such thiosulfate-containing developing compositions are used in the development of photographic paper, a more or less pronounced yellow to brown fog is produced, depending on the type and age of the photographic paper. In the presence of some stabilizers, e.g., 1-phenyl-5-mercapto-tetrazole, this fog may also be colored blue to blue violet. This fog consists of finely divided silver deposited in the baryta layer.

In barytes coated photographic papers, this yellow fog is due to silver salts which migrate during casting from the emulsion into the barytes layer where they are retained by adsorption. On storage of these finished papers, these silver salts are reduced to silver, a process which takes place particularly in the first months of storage. If silver halide solvents such as thiosulfates are added to the developer during the processing of the papers, the dissolved silver salts are reduced on the silver nuclei of the barytes-coating, and yellow fog and patches are produced.

After storage, the yellow fog is particularly pronounced on areas of the paper previously exposed to atmospheric moisture, e.g., at the edges of the paper and on the top sheet of a package.

2

The yellow fog occurs particularly when unrinse emulsions of silver chloride or of silver chlorobromide are used because the chlorides present in excess can form soluble silver complex salts.

5 The yellow fog also occurs if types of gelatin containing compounds that dissolve silver halide are used in the production of the emulsion or of the baryta layer and if in addition there are present degradation products of gelatin which forms nuclei. These types of gelatin also 10 produce a yellow fog in photographic films.

In addition, emulsions that have not been fully ripened and which have a steep gradation also tend to produce a yellow fogging, especially if high-contrast-developers with a high content of potassium bromide are used for 15 developing the latent silver image.

It is among the object of the invention to provide stabilizers prevent the formation of any fog in photographic materials without concomitant undesired effects on the photographic properties. Another object of the 20 invention is the production of photographic materials containing these agents.

We now have found a photographic material with at least one silver halide emulsion layer, which material contains benzimidazole - 2 - thione-N,N'-dicarbonic acid 25 esters.

Particular utility is exhibited by compounds of the following formula:



35 wherein represents:

R<sup>1</sup> straight-chain or branched alkyl having up to 6 C atoms;

R<sup>2</sup> hydrogen, halogen preferably fluorine, chlorine or 40 bromine, alkyl having up to 6 carbon atoms which may be substituted e.g. with halogen such as in the trifluoromethyl group, alkoxy having up to 6 carbon atoms, aroxy in particular phenoxy, nitro, carboxy, carbamoyl, sulfo or sulfamoyl and

45 n 1 or 2.

The compounds shown in the following table have been found to be especially suitable.

TABLE

| Compound Number: | R <sup>1</sup>                                     | R <sup>2</sup>     |
|------------------|----------------------------------------------------|--------------------|
| 1                | —C <sub>2</sub> H <sub>5</sub>                     | H                  |
| 2                | —C <sub>2</sub> H <sub>5</sub>                     | 5,6-Cl             |
| 3                | —C <sub>2</sub> H <sub>5</sub>                     | 5-OCH <sub>3</sub> |
| 4                | —CH <sub>2</sub> —CH <sub>2</sub> —CH <sub>3</sub> | 5-Cl               |
| 5                | —CH(CH <sub>3</sub> ) <sub>2</sub>                 | 5,6-Cl             |
| 6                | —CH <sub>2</sub> —CH <sub>2</sub> —CH <sub>3</sub> | 5,6-Cl             |
| 7                | —C <sub>2</sub> H <sub>5</sub>                     | 5-Cl               |
| 8                | —C <sub>2</sub> H <sub>5</sub>                     | 5-NO <sub>2</sub>  |

60 The compounds to be used according to the invention are prepared by reacting the benzimidazole-2-thione from which they are derived with pyrocarbonic acid esters, preferably in diluents.

#### PREPARATION OF COMPOUND 1

65 150 g. (1 mol) of 2-mercaptopbenzimidazole, 500 ml. of ethanol and 405 g. (2.5 mol) of diethylpyrocarbonate are gradually heated to 50° C. and kept at this temperature until they dissolve. On the next day, 1.3 l. of petroleum ether are added, the reaction mixture is cooled for some time at —20° C. and the crystalline product obtained is removed by suction filtration and washed with petroleum ether which has been cooled to a low tempera- 70

ture. The crude product (187 g. M.P. 30 to 42° C.) is purified by dissolving it in a lukewarm mixture of 470 ml. of ethanol and 1.4 l. of petroleum ether, clarifying with charcoal and cooling to 0° C. with stirring, and the diethylester of benzimidazoline-2-thione-N,N'-dicarboxylic acid which precipitates is isolated. The product is now completely pure and melts at 65.5 to 66° C.

#### PREPARATION OF COMPOUND 2

21.9 g. (0.1 mol) of 2-mercaptop-5,6-dichlorobenzimidazole, 40 ml. of ethanol, 48.6 g. (0.3 mol) of diethylpyrocarbonate and 0.5 ml. (0.001 mol) of 2 N sodium methylvate solution are kept stirred overnight. The sandy reaction product obtained is removed by suction filtration (33.7 g., M.P. 109 to 113° C.) and recrystallised from ethanol. 25.5 g. of pure compound are obtained. M.P. 113-114° C.

#### PREPARATION OF COMPOUND 3

A suspension of 72.0 g. (0.4 mol) of 2-mercaptop-5-methoxybenzimidazole and 388.8 g. (2.4 mol) of diethylpyrocarbonate is heated on a bath at a temperature of 90° C. A vigorous exothermic reaction sets in after about 2 hours, and at that moment the bath is removed. When the reaction has died down, the reaction mixture is again heated for 1½ hours on a bath which is at a temperature of 90° C. 400 ml. of ethanol are then added and the reaction mixture is then inoculated and left at -20° C. for complete crystallisation. The crystalline product is then removed by suction filtration and washed with deep cooled ethanol. 94.4 g. of the diethylester of 5-methoxybenzimidazoline - 2 - thione-N,N'-dicarboxylic acid, M.P. 76.5 to 77° C. are thus obtained. The product is purified by dissolving it in 4 times its quantity of hot ethanol, clarifying with charcoal and precipitating with 4 times the volume of hot light fraction petroleum hydrocarbons. The product then melts at 77.5 to 78° C.

#### PREPARATION OF COMPOUND 4

9.23 g. (0.05 mol) of 2-mercaptop-5-chlorobenzimidazole, 20 ml. of n-propanol, 0.1 g. of the sodium salt of mono-n-propyl-carbonate and 28.5 g. (0.15 mol) of di-n-propylpyrocarbonate are stirred together, a solution being soon formed with evolution of CO<sub>2</sub>. On the next day, 70 ml. of petroleum ether are added and the reaction mixture is cooled to -20° C. and inoculated, and the product which then precipitates is removed by suction filtration after some time (3.4 g., M.P. 56 to 57° C.). After recrystallisation from petroleum ether (deep cooling) the product has a sharp melting point of 57° C.

#### PREPARATION OF COMPOUND 5

10.95 g. (0.05 mol) of 2-mercaptop-5,6-dichlorobenzimidazole, 20 ml. of isopropanol, 0.1 g. of the sodium salt of monoisopropylcarbonate and 28.5 g. (0.15 mol) of diisopropyl pyrocarbonate are stirred together. A reaction sets in and CO<sub>2</sub> is evolved. On the next day, the product is removed by suction filtration after it has been cooled to -20° C. and is then recrystallized from isopropanol. 12.0 g., M.P. 127.5 to 128° C., are obtained.

#### PREPARATION OF COMPOUND 6

10.95 g. (0.05 mol) of 2-mercaptop-5,6-dichlorobenzimidazole, 20 ml. of n-propanol, 0.1 g. of the sodium salt of mono-n-propylcarbonate and 28.5 g. (0.15 mol) of di-n-propylpyrocarbonate are stirred together, the original suspension being converted into the reaction product with evolution of CO<sub>2</sub>. On the next day, the crude product is removed by suction filtration at 0° C. (14.8 g., M.P. 80 to 80.5° C.) and recrystallized from acetonitrile. The compound then melts at 80.5 to 81° C.

#### PREPARATION OF COMPOUND 7

46.1 g. (0.25 mol) of 2 - mercapto-5-chlorobenzimidazole. 135 ml. of ethanol, 97.2 g. (0.6 mol) of diethyl-

pyrocarbonate and 1.25 ml. of 2 N sodium methylvate solution are stirred together. A reaction sets in with evolution of CO<sub>2</sub>. On the next day, the product is removed by suction filtration and purified by recrystallisation from ethanol. 40.3 g. (M.P. 88.5 to 89° C.) are obtained.

#### PREPARATION OF COMPOUND 8

5 58.5 g. (0.3 mol) of 2-mercaptop-5-nitrobenzimidazole and 243 g. (1.5 mol) of diethylpyrocarbonate are heated 10 in an oil bath which is at a temperature of 100° C. until they dissolve (2 hours). A paste is formed on cooling. It is removed by suction filtration at 0° C. and washed with alcohol. The resulting crude diethylester of 5-nitrobenzimidazoline - 2 - thione-N,N'-dicarboxylic acid, melting 15 point 135° C., is purified by recrystallizing it twice from 5 times its quantity of toluene. The product then melts at 138 to 138.5° C.

The photographic materials are prepared in accordance with common practice including the steps of:

20 (1) Precipitation of the silver halide in the presence of a protective colloid and physical ripening;

(2) If desired removal as by washing from the resulting emulsion, the excess water-soluble salts that have formed as a result of the precipitation;

25 (3) Chemical ripening (after-ripening) the washed product to impart the desired sensitivity to the emulsion; and

(4) Applying the emulsion on a suitable support and drying.

30 The bisimidazoline compounds of the present invention can be added to any photographic layer within the photographic material. Preferably the stabilizers are added to a silver halide emulsion layer or to the baryta-coating depending somewhat on the desired effect. If fog inhibition in the silver halide emulsion layer is desired they are added preferably to an emulsion layer. On the other hand if the formation of yellow fog in the baryta-coating is to be prevented the stabilizers are preferably added to the baryta-coating. The stabilizers of the present invention, however, can also be incorporated into any other auxiliary photographic layer since in any case the compounds diffuse into the other layers of the photographic material during development. The auxiliary layers may be water-permeable intermediate layer protective layers or as in the silver salt diffusion process it may also be an image-receiving layer.

35 It depends on the desired effect and the photographic material to which layer the compound is to be added to obtain the optimum effect. This, however, can be found out easily by simple experiments customarily employed in the art.

40 The stabilizers can be added to the photographic layers at any stage of their production. They are added to the silver halide emulsions preferably after the chemical ripening to the casting solution for the emulsion layer. It is, however, also possible to add the stabilizers to the silver halide emulsion before chemical ripening.

45 The same holds true if they are to be added to the baryta-coating. Also in this case they can be added at any stage of the production of the baryta layer; for example: before, during or after heating or mixing the baryta suspension.

50 The benzimidazoline compounds can be used in any silver halide emulsion. Suitable silver halides for the emulsion are silver chloride, silver bromide or mixtures thereof, if desired containing up to 10 mols-percent of silver iodide. The silver halides may be dispersed in the usual hydrophilic compounds such as carboxymethyl cellulose, polyvinyl alcohol, polyvinylpyrrolidone, alginic acid and its salts, esters or amides or, preferably, gelatin.

55 The methods of incorporating the compounds in the photographic layers are relatively simple and well-known to those skilled in the photographic art. It is convenient to add the stabilizers from solutions in appropriate sol-

vents whereby the solvent should be completely free from any deleterious effect on the ultimate light-sensitive material. Suitable are in particular solvents miscible with water such as methanol, ethanol alone or in admixtures, tetrahydrofuran or acetone.

The concentration of the stabilizers in the layers can vary widely, for instance from about 1 mg. to 0.5 g., preferably 22-200 mg. per mol silver halide. In the baryta-coating the compounds are added in amounts of 0.01 to 2.0 g., preferably 0.1 to 1.0 g. per kg. barium sulfate. The optimum concentration depends on the type of the layer and on the effects desired. The optimum concentration will be apparent to those skilled in the art upon making the tests and observations customarily employed in the art.

The emulsions can also be optically sensitized with cyanine, rhodacyanine or merocyanine dyes such as described by F. M. Hamer "The Cyanine Dyes and and related Compounds," Interscience Publishers, (1964).

The emulsions may also contain chemical sensitizers, e.g. reducing agents such as stannous salts, polyamines such as diethyltriamine or sulfur compounds as described in U.S. Pat. No. 1,574,944. For chemical sensitization, one may further add to the given emulsions salts of noble metals such as ruthenium, rhodium, palladium, iridium, platinum or gold, as described in the article by R. Koslowsky, Z. Wiss. Phot. 46, 65-72 (1959). The emulsions may also contain polyalkylene oxides, especially polyethylene oxide, and derivatives thereof, as chemical sensitizers.

The silver halide emulsions may additionally contain the usual stabilizers, e.g. homopolar or salt-type compounds of mercury with aromatic or heterocyclic rings, such as mercaptotriazoles, simple mercury salts, sulfonium mercury double salts, and other mercury compounds. Other stabilizers which may be used include azaindenes, especially tetra- or penta-azaindenes, in particular those substituted with hydroxy or amino groups. Compounds of this type have been described in the article by Birr, Z. Wiss. phot. 47, 2-58 (1958). Other suitable stabilizers include heterocyclic mercapto compounds, e.g. 1-phenyl-5-mercapto - tetrazole, quaternary benzthiazole derivatives and benztriazoles.

The photographic layer may be hardened in the usual manner, for example, with formaldehyde or halogen-substituted aldehydes that contain a carboxyl group, e.g. mucobromic acid, diketones, methanesulfonic acid esters and dialdehydes.

The stabilizers which we have described may be used in various kinds of photographic emulsions. In addition to being useful in X-ray and other non-optically sensitized emulsions they may also be used in ortho-chromatic, panchromatic and infrared-sensitive emulsion. They may also be used for emulsions suitable for use in the silver salt diffusion process for color-photographic emul-

phenylolpropane or opaque supports such as paper, in particular baryta-coated paper which may be provided with hydrophobic layers of, for example, polyolefines such as polyethylene or polypropylene.

The photographic materials can be processed by the usual processing techniques. Any photographic developer or developer combination is operative for developing the exposed photographic material. The developer compounds can be added to a photographic layer or to the aqueous processing bath. For example, it is possible to use developers of the hydroquinone type, pyrocatechol type, p-methylaminophenol, compounds of the 1-phenylpyrazolidone-3 series or phenylenediamine developers. The following examples illustrate the invention:

#### Example 1

A very highly sensitive silver iodobromide emulsion containing 5 mols percent of silver iodide is prepared in the usual manner, the silver nitrate being introduced at intervals into a solution which contains gelatin in addition to KI and KBr. The emulsion is flocculated with ammonium sulfate in a known manner and freed from the soluble salts.

The flocculate is redispersed in warm water and the required quantity of gelatin which contains sulfur is added. The emulsion is then divided into several parts, the first part containing no additive whereas a stabilizer is added to each of the other parts. Noble metal salts, preferably gold salts, are then added to all the samples of emulsion and the samples are ripened to their optimum sensitivity.

The emulsions are then prepared ready for casting by the addition of 200 mg. of 4-hydroxy-6-methyl-1,3,3a,7-tetraazaindene as stabilizer, 600 mg. of saponin as wetting agent and 10 ml. of 10 percent aqueous solution of formaldehyde, the amounts being in each case based on 1 kg. of emulsion. The emulsion is cast on a layer support of cellulose acetate. Some of the film samples are stored at 60° C. for 3 days.

After exposure in a sensitometer customarily employed in the art behind a step wedge, the emulsion layers are developed in a developer of the following composition:

|    |                                 | G.   |
|----|---------------------------------|------|
| 45 | Sodium sulfite anhydrous        | 70.0 |
|    | Borax                           | 7.0  |
|    | Hydroquinone                    | 3.5  |
|    | p-Monomethylaminophenol sulfate | 3.5  |
| 50 | Sodium citrate                  | 7.0  |
|    | Potassium bromide               | 0.4  |
|    | Made up with water to 1 l.      |      |
|    | Developer temperature: 20° C.   |      |

The results of the sensitometric test are shown in the following table.

TABLE

| Substance number | Quantity in mg. | 7' development time |          |      | 16' development time |          |      | 3 days heating, 7' development time |          |      |
|------------------|-----------------|---------------------|----------|------|----------------------|----------|------|-------------------------------------|----------|------|
|                  |                 | S, degree           | $\gamma$ | Fog  | S, degree            | $\gamma$ | Fog  | S, degree                           | $\gamma$ | Fog  |
| Blank            | (1)             |                     |          |      |                      |          |      |                                     |          |      |
| 1                | 5               | +0.5                | 0.85     | 0.28 | ±0                   | 1.25     | 0.41 | ±1.0                                | 1.10     | 0.54 |
| 2                | 3               | -1.0                | 1.00     | 0.28 | -0.5                 | 1.35     | 0.32 | ±0                                  | 1.25     | 0.38 |
| 3                | 5               | +1.0                | 1.30     | 0.28 | +0.5                 | 1.40     | 0.32 | +1.0                                | 1.50     | 0.40 |
| 6                | 3               | +1.0                | 1.10     | 0.24 | +1.0                 | 1.40     | 0.30 | +1.0                                | 1.50     | 0.40 |
| 7                | 3               | +1.0                | 1.30     | 0.26 | +1.0                 | 1.60     | 0.32 | ±0                                  | 1.70     | 0.40 |

<sup>1</sup>No additive.  
NOTE.—S=sensitivity;  $\gamma$ = $\gamma$ -value; (3°=1 shutter stop).

sions and for photographic materials for the silver dye bleach process.

The photographic material may comprise any kind of support customarily used for photographic materials. Suitable supports are, for example, transparent films of cellulose esters such as cellulose acetate, of polyesters in particular on the basis of polyethyleneglycol-terephthalic acid, of polycarbonates, preferably on the basis of bis-

#### Example 2

An unrinsed silver chlorobromide gelatin emulsion (20 mol-percent silver bromide) containing per litre 0.18 mol silver halide, 20 ml. of a 10% aqueous solution of saponine and 2 ml. of a 30% aqueous solution of formaldehyde is divided into several parts. To each sample is added a stabilizer of the present invention in form of a

